

Jan. 3, 1928.

1,654,817

A. KADOW

PROCESS OF MANUFACTURING GLASS

Filed Nov. 16, 1923

2 Sheets-Sheet 1



Fig 1

INVENTOR

AUGUST KADOW.  
Owner, Owen & Crampton

attorneys

Jan. 3, 1928.

1,554,817

A. KADOW

PROCESS OF MANUFACTURING GLASS

Filed Nov. 16, 1923

2 Sheets-Sheet 2



Inventor

AUGUST KADOW.

By Owen, Owen & Crampton

Attorney's

## UNITED STATES PATENT OFFICE.

AUGUST KADOW, OF TOLEDO, OHIO, ASSIGNOR TO THE LIBBEY GLASS MANUFACTURING COMPANY, A CORPORATION OF OHIO.

## PROCESS OF MANUFACTURING GLASS.

Application filed November 16, 1923. Serial No. 675,052.

My invention relates to the manufacture of glassware, and has for its object the improvement of the ware and the simplification and speeding up of the process of manufacture.

Features of my invention are capable of general use, but the invention is particularly applicable to the production of hollow ware that is blown with a moil which differs in thickness from the walls of the finished articles. I will describe my invention as applied to the manufacture of blown tumblers, and particularly as combined with the process described and claimed in the copending joint application of applicant and Alvah C. Parker, Serial No. 704,571, filed April 7, 1924.

The process of manufacturing tumblers now in general use is to first anneal the tumblers with the moil thereon, an operation which consumes several hours. After annealing, the obviously defective articles are thrown out and the moil is cracked off of the apparently good articles. This is usually done by making a scratch on the desired line of severance and then applying heat to that line, producing strains that result in cracking the glass, usually along the desired line, but sometimes along undesired lines.

The edge of the tumbler is left rough by the cracking off process, and is smoothed by grinding during which there is considerable loss from breakage. Grinding leaves the tumbler wet and dirty, and it is cleaned and dried before the next operation. The ground edge has sharp corners and is unglazed. To round the corners and glaze the edge, a glazing or fire finishing flame is played upon the edge of the tumbler. As the edge of the tumbler must be melted while the body of the tumbler is left comparatively cold, strains are set up which remain in the finished article permanently, or until breakage results. The only way to relieve such strains would be by re-annealing after fire finishing.

The attached moil is usually of more irregular thickness than the body of the article. Because of this, cooling the article with the moil thereon sets up strains, unless this cooling is done very slowly and care-

fully. The annealing process is greatly lengthened because of the slow heating and cooling required to avoid breakage, the extra strains introduced by the presence of the moil, and the comparatively low maximum annealing temperature customarily employed to avoid too great a range through which heating and cooling must be carried.

The moil has been cracked-off of un-annealed electric light bulbs with some degree of success, though the percentage of breakage was high; but with ware heavy enough to be used as open-mouthed articles, it has been considered impracticable to crack-off the moil before annealing because of the very great percentage that would crack along lines departing widely from the intended line of severance.

My improved process is as follows, reference being had to the accompanying drawings, in which Fig. 1 is a diagrammatic view illustrating the complete process and Figs. 2 and 3 are diagrammatic views of one step in the process.

A glass batch is gradually charged into a melting tank A. As the batch is melted, the molten glass flows into a refining chamber B, and from the refining chamber to a working chamber C. I prefer to keep the glass in the refining chamber cooler than proper working temperature, and heat the chamber C so that the temperature of the glass is gradually raised as it flows into the working chamber and passes to the working point. It is easier to maintain the glass at the working point substantially uniform in temperature and consistency when the refined glass is heated to a higher temperature while it passes to the working point than it is when the refined glass cools as it approaches the working point.

Uniformity of temperature and consistency of the glass at the working point results in fewer strains within the formed articles, facilitating subsequent operation and producing better ware.

The glass is worked out of the tank C, and blown, as at D, preferably by an automatic gathering and blowing device.

The articles are dropped from the blowing machine onto a carrier E, from which

they are taken and placed in an apparatus F, where the moil is burned off. I prefer to pass the articles from the molds to the burning off apparatus with as little cooling as possible. The burning off apparatus may be constructed in any suitable manner.

The burning off process consists in the application of a sharp thin flame along the desired line of severance to melt a ring of 10 glass, and the pulling off of the moil by its own weight or otherwise. After severance is completed, I prefer to continue the melting flame for a time a short distance from the severed edge, to melt off any stringing glass 15 and smooth up the edge, but this finishing action may be produced by any other suitable application of heat.

Some of the glass which is melted to effect the severance remains on the severed 20 edge, and surface tension gives this glass the form of a bead along the severed edge. The shape of the bead may be modified and controlled as more fully described in the above identified copending application.

25 Figs. 2 and 3 illustrate diagrammatically the bead forming step. In Fig. 2 there is shown a tumbler 10, supported in a chuck 11 carried by a shaft 12 rotated by a friction wheel 13 contacting the face of a driving friction wheel 14. The wheel 13 may be slidably keyed onto the shaft 12, and moved by handle 15 radially of driving wheel 14 to regulate the speed of rotation of the chuck.

35 An annular burner 16 is provided for melting off the moil 17. The chuck may be rotated with such speed that the molten glass on the severed edge is moved outward by centrifugal force to form an outwardly extending bead, 40 as shown at 18 in Fig. 2. The chuck may be rotated comparatively slowly by moving wheel 13 nearer the center of wheel 14, as shown in Fig. 3, and the flame may be so regulated that the article 19, shown in that 45 figure, will have an inwardly projecting bead 20. Preferably, an intermediate speed is chosen, and the bead is placed symmetrical- ly on the severed edge.

There is a tendency for glass of substan- 50 tially equal thickness throughout to heat and cool more rapidly at the exposed edges. A thickened bead along the edge tends to make the temperature changes of the edge more nearly equal to those of the adjacent sides, 55 and this is an advantage in annealing, as it makes possible more rapid changes in the temperature of the article without causing detrimental temperature-differences between the edge and the adjacent glass.

60 Where a hot glass article is placed in burning off apparatus, the chuck or other member contacting the article must be of non-conducting material, or else heated, in order to avoid breakage or strain in the article. Preferably, the article is not only

70 prevented from cooling during the burning off process, but the chuck holding the article is heated, and that, with the rising heat from the burning off and fire finishing flame, heats the article nearly to annealing tem- 75 perature, or about as hot as it can be han- dled without danger of deformation. Where necessary, additional heat may be applied to exposed portions of the article during the burning off and finishing processes. In 75 Figs. 2 and 3 a burner 21 is shown for heat- 80 ing the chuck and article therein. In this way there is the least possible strain intro- duced by differential temperature between the burned off edge and the body of the 80 article.

The articles are taken from the burning off apparatus and placed in an annealing 85 leer G. The leer may be of any suitable type, but I prefer to use a muffle tunnel leer. 85 I prefer to use a temperature higher than that usually employed in the entrance end of the leer so that the articles are heated to a high annealing temperature within a short 90 time.

Annealing is for the purpose of allowing 95 re-arrangement of molecules to relieve strains caused by a varying consistency of 100 glass and differential temperatures or rates of cooling. This re-arrangement takes place 95 scarcely at all below what is termed the criti- 105 cal temperature, which approaches that at which the glass may be permanently de- formed under pressure; and the rate of the 110 re-arrangement increases rapidly as the tem- 110 perature is raised above this point. I prefer 115 to heat the glass as hot as possible without 120 having it suffer change of shape, in order to shorten the annealing period. I can apply 125 sufficient heat to quickly raise the tempera- 130 ture of the glass to a high annealing point 135 because the articles enter the leer at nearly 140 annealing temperatures, so that the applica- 145 tion of heat will not crack them even where 150 the walls are not of uniform thickness, as 155 where the bottoms of tumblers are thicker 160 than their sides, for example.

The necessary duration of annealing is, of 165 course, proportional to the strains which are 170 introduced into the ware, and so the uniform 175 character of the glass at the gathering point 180 tends to reduce the time necessary for annealing. Likewise, the absence of cooling 185 between blowing and annealing avoids the 190 introduction of cooling strains, and so elimi- 195 nates the necessity for long annealing to re- 200 move such strains. The speed with which 205 the temperature of the article may be safely 210 changed, both in heating and cooling, is 215 much greater with an article having walls of 220 comparative uniform thickness than it 225 would be with an article having a moil of 230 uneven thickness attached thereto. After 235 the glass is cooled down below the critical 240 point, further cooling may be very rapid, 245

as no permanent strains will be set up by such cooling.

To summarize, shortening of the time of annealing is aided and accomplished by the uniform consistency of glass at the working point, the avoidance of cooling strains after blowing, the comparatively high temperature at which the articles are introduced into the leer and the comparatively uniform thickness of walls resulting from the removal of the moil, the high temperature at which the annealing is done, and the speed with which the articles are cooled after passing below annealing temperature. As a result of these combined features, I have passed tumblers through the leer in less than eight minutes with very satisfactory results.

It is possible, and under some circumstances even preferable, to heat the articles sufficiently during the burning off process so that no further removal of strains is necessary, and the articles may be transferred at once to heated or non-conducting receptacles, or other means may be used to prevent too rapid cooling until they are below the critical temperature.

The articles are taken from the leer and inspected on a carrier H and packed, as at I, one of the important features of my invention being that the articles leave the leer in finished form and no subsequent strain introducing processes are necessary. As will be seen, I substitute a burning off step for cracking off, grinding, washing and fire finishing, and greatly shorten the time of annealing, lessening the original cost of the plant and eliminating most of the workmen required. At the same time the article, which may be packed within twelve minutes of its removal from the blow mold, does not have internal strains introduced by processes subsequent to annealing, and has a beaded edge, if desired.

While I have described my process as applied to blown tumblers, it is obvious that other articles could be made by a similar process; and while all of the described steps co-operate in producing the desired result in the manufacture of blown tumblers and similar ware, it is obvious that less than the complete process could be applied with beneficial results. For example, the described method of obtaining uniform glass at the working point is useful in making quick annealing possible with ware where there is no removal of moil or severance of the article between shaping and annealing. Furthermore, dividing by burning off before annealing is especially useful where a moil is removed from a blown article and where the burning off step is utilized to heat the article to proper temperature to enter the annealing zone; but it is useful in producing a properly finished annealed edge on the completed article, however the glass is initially

shaped and however the annealing after dividing is done.

Other variations, within the scope of the appended claims may be made in the described process without departing from the spirit of the invention.

It will be understood that, in the appended claims, where the terms "final form" and "finished shape" are used, it is intended to distinguish from such an article as an electric light bulb as it leaves the glass factory, before the filament and base have been inserted and the final form has been given. My process, and particularly the annealing step, is pertinent where the ware is thick enough so that the severed edge may be permanently exposed during the useful life of the article.

What I claim is:

1. In the manufacture of glassware, the process which consists in forming a set shape of molten glass, severing the set glass by melting it along the line of severance so quickly that severance results and leaves the glass constituting the severed edge of the finished article in substantially its original position with regard to the portion of said article to which it is attached, and thereafter raising the temperature of the glass for annealing purposes, and finally allowing it to cool.

2. In the manufacture of glassware, the process which consists in blowing a glass article, removing the moil by melting the glass along the line of severance so quickly that severance results and leaves the glass constituting the severed edge of the finished article in substantially its original position with regard to the portion of the article to which it is attached, and thereafter annealing the article.

3. In the manufacture of a glass article having an edge which is exposed during the normal use of the article, the process which consists in forming a set shape for molten glass, severing the set glass by melting it along a desired line to form said exposed edge of the finished article, and thereafter annealing the article.

4. In the manufacture of a blown glass article having an edge which is exposed during the normal use of the article, the process which consists in blowing the article with a moil attached, severing the moil from the article by melting the glass along the desired line of severance to form the exposed edge of the finished article, and thereafter annealing the article.

5. In the manufacture of a blown glass article having an edge which is exposed during the normal use of the article, the process which consists in blowing an article with a moil attached, removing the moil by melting the glass along the line where said edge is to be formed, the melting being performed

so quickly that severance results and leaves the glass constituting the severed edge of the finished article in substantially its original position with regard to the portion of the 5 said article to which it is attached, and thereafter annealing the article.

6. The process of manufacturing blown open-mouthed glass article, which consists in blowing such an article with a moil attached, 10 melting off the moil to give the article final form, and thereafter passing the article through an annealing leer, bringing the entire article to a high annealing temperature within a period of not more than ten minutes 15 after it enters the leer and cooling it so that it may be removed from the leer within a period not more than one-half hour after it enters the leer.

7. In the manufacture of glassware, the 20 process which consists in melting a batch to form molten glass, refining the glass at a comparatively low temperature, reheating the refined glass, shaping the reheated glass to give it the desired form of the finished 25 article, and annealing without allowing it to become cool after shaping, and completing the annealing within one-half hour after shaping.

8. In the manufacture of glassware, the 30 process which consists in dividing a glass article by applying heat intense enough to melt the glass along a desired line of severance and leave a severed edge along said line, and heat treating the article so that all 35 portions of it will be at approximately the critical temperature upon the completion of severance.

9. In the manufacture of glassware, the 40 process which consists in dividing glass by applying heat intense enough to melt the glass along a desired line and leave a severed edge along said line, fire finishing the severed edge, and heat treating the article so that all 45 portions of it will be at approximately the critical temperature upon the completion of fire finishing.

10. In the manufacture of glassware, the 50 process which consists in forming a set shape from molten glass, directly thereafter melting the shape along a desired line of severance by means of a flame so intense that it severs the glass and leaves a severed edge along the line of its application and thereby gives the final form to the article, forming 55 a bead along the severed edge at the time of severance, and heat treating the article so that all portions of it will be at approximately the critical temperature when severance is completed.

60 11. In the manufacture of a glass article having an edge which is exposed during the normal use of the article, the process which consists in forming a set shape from molten glass, severing said shape by melting the 65 glass along the desired line of severance so

quickly that severance results and leaves the glass constituting the severed edge in its original position with regard to the portion of said article to which it is attached, except for a small amount of glass which is melted and forms a bead along said severed edge, said severed edge forming the exposed edge of the finished article, and thereafter raising the temperature of the glass and annealing the article.

70 12. In the manufacture of glassware, the process which consists in blowing an article, melting off the moil along a line by means of a flame so intense that it severs the glass and leaves a severed edge along the line of its application and thereby gives the article 80 its finished form, forming a bead along the severed edge during the severing process, and heat treating the article so that all portions of it will be at approximately the 85 critical temperature when severance is completed.

90 13. In the manufacture of a blown glass article having an edge which is exposed during the normal use of the article, the process which consists in blowing an article with a moil thereon, severing the moil from the article by melting the glass along the desired line of severance so quickly that severance results and leaves the glass constituting the severed edge of the finished article in its original position with regard to the portion of the said article to which it is attached, except for a small amount of glass 95 which is melted and forms a bead along said severed edge, heat treating the article so that all portions of it will be at approximately the critical temperature when severance is completed, and thereafter retaining the heat for annealing purposes.

100 14. In the manufacture of glassware, the process which consists in blowing an article, removing the moil by melting the glass along a line of severance by means of a flame so intense that it severs the glass and leaves a severed edge along the line of its application and thereby gives the finished form to the article, fire finishing the severed edge, forming a bead along the edge during severance and fire finishing, and heat treating the article so that all portions of it will be at approximately the critical temperature when fire finishing is completed.

110 15. In the manufacture of glassware, the process which consists in blowing an article, removing the moil by melting the glass along a line of severance by means of a flame so intense that it severs the glass and leaves a severed edge along the line of its application and thereby gives the finished form to the article, finishing the severed edge, forming a bead along the edge during severance and fire finishing, and heat treating the article so that all portions of it will be at approximately the critical temperature 120 125 130

when fire finishing is completed, and thereafter retaining the heat for annealing purposes.

16. In the manufacture of a blown glass article having an edge exposed during the normal use of the article, the process which consists in blowing an article with moil attached, removing the moil by melting the glass along the desired line of severance.

10 fire-finishing the severed edge and forming

a bead thereon while contacting it by gases only, heat treating the article so that all portions of it are at approximately the critical temperature when bead formation is completed, thereafter quickly raising the temperature of the article to high annealing heat, and finally cooling the article.

In testimony whereof, I have hereunto signed my name to this specification.

AUGUST KADOW